

Feb. 13, 1923.

1,444,799

J. J. McCABE

CORSET BONING AND METHOD OF MAKING THE SAME

Filed Apr. 2, 1921



Inventor.

John J. McCabe  
by Merrill C. Clark  
His Attorney

## UNITED STATES PATENT OFFICE.

JOHN J. McCABE, OF BRIDGEPORT, CONNECTICUT, ASSIGNOR TO THE WARNER BROTHERS COMPANY, OF BRIDGEPORT, CONNECTICUT, A CORPORATION OF CONNECTICUT.

## CORSET BONING AND METHOD OF MAKING THE SAME.

Application filed April 2, 1921. Serial No. 453,017.

*To all whom it may concern:*

Be it known that I, JOHN J. McCABE, a citizen of the United States, residing at Bridgeport, in the county of Fairfield, State 5 of Connecticut, have invented a new and useful Corset Boning and Method of Making the Same, of which the following is a description.

My invention relates to corset boning 10 made of steel or similar material.

The general object of my invention is to provide boning of that character, with a covering which will render it rust-proof and at the same time will cause it to simulate 15 genuine whalebone.

Another object of my invention is to provide a covering for corset boning which will not crack or peel off in use, nor stain the garment with which it may be in contact.

With these and other ends in view, as 20 will appear more fully hereinafter, my invention includes the novel method, steps and article described herein and more particularly defined in the appended claims.

Referring to the accompanying drawing:—

Fig. 1 shows a piece of steel ribbon such as is ordinarily used for corset boning;

Fig. 2 shows a paper ribbon of such dimensions that it will completely encase the steel ribbon.

Fig. 3 shows the steel ribbon in the process of being encased in the paper ribbon;

Fig. 4 shows the paper encased steel ribbon;

Fig. 5 is a more or less diagrammatic view showing the method which I preferably employ for coating or impregnating the paper encased steel ribbon to produce 40 the finished boning; and

Fig. 6 shows a finished corset bone cut to the desired length.

In carrying out my improved method, I preferably start with a steel ribbon such as 45 shown at A in Fig. 1, and of indefinite length, since I find it more convenient to cut the boning into desired lengths after the operations that I am about to describe have been completed rather than before.

This steel ribbon A I encase in paper, preferably in the form of a paper ribbon B (Fig. 2). I preferably accomplish this in

the manner illustrated in Fig. 3, although obviously it may be done in other ways. The paper surrounding the steel ribbon is 55 glued, cemented or otherwise secured thereto in such a way as to make a substantially unitary structure, such as shown in Fig. 4.

The next step in my improved process is the coating or impregnating step. This 60 may be accomplished in several different ways, but I prefer to do it in the manner indicated more or less diagrammatically in Fig. 5. As shown in this figure, the paper encased steel ribbon is led off of a supply 65 reel C, whence it passes about a roller or similar device D, in the liquid container E. The liquid in this container is preferably a black celluloid solution, and I find that excellent results are obtained from such a 70 solution comprising celluloid (for example, waste celluloid) dissolved in suitable acetones or acetates.

In passing out of the container E the ribbon preferably passes through a wiper F, of 75 suitable form, for removing the excess liquid.

After passing through the wiper F the ribbon passes through a drying compartment G which may be heated in any desired manner. From the drying chamber 80 the ribbon passes to the winding reel H from which it may be removed, when desired, and cut into proper lengths. After being cut the ends of the corset bones or 85 steels thus formed are preferably finished by first covering them with metal tips, and then dipping them into a liquid such as that contained in the container E, and then drying them. The finished corset bone or steel 90 is represented in Fig. 6.

I have found from experience that the corset boning produced as above described answers all requirements of service in a most satisfactory manner and is far superior to 95 any artificial boning heretofore known. I attribute the success of this boning largely to my use of paper as an encasing material, and to the fact that the affinity between the paper and the celluloid solution is exactly 100 of the order required to produce the most beneficial results. The impregnated paper cover is impervious to moisture and, accordingly, my improved boning is rust-proof.

Also, the surface formed by the impregnated paper is very similar to the surface of natural whalebone, both in appearance and to the touch.

5 It is evident, therefore, that I have produced an artificial corset boning which not only has all of the advantages of the natural article from the standpoint of utility, but which also resembles the natural article in 10 appearance far more closely than do any of the prior artificial bonings with which I am familiar.

15 The terms and expressions which I have employed are used as terms of description and not of limitation, and I have no intention, in the use of such terms and expressions, of excluding any equivalents of the features shown and described, or portions thereof, but recognize that various modifications 20 are possible within the scope of the invention claimed.

What I claim is:

1. Corset boning comprising a ribbon-like piece of steel encased in celluloid coated 25 paper.

2. Corset boning comprising a ribbon-like piece of steel encased in paper which is coated with a solution of celluloid in acetone.

30 3. The method of making corset boning which consists in encasing a ribbon-like piece of steel in a covering of paper, and then immersing the paper encased steel in a celluloid solution.

35 4. The method of making corset boning which consists in encasing a ribbon-like piece of steel in a covering of paper, caus-

ing the paper to adhere to the steel, and then immersing the paper encased steel in a celluloid solution.

40 5. The method of making corset boning which consists in encasing a ribbon-like piece of steel in a covering of paper, immersing the paper encased steel in a liquid celluloid solution, and finally drying it by subjecting it to heat.

45 6. The method of making corset boning which consists in encasing a ribbon-like piece of steel in a covering of paper, and then immersing the paper encased steel in a solution of celluloid dissolved in acetone.

50 7. The method of making corset boning which consists in encasing a ribbon-like piece of steel in a covering of paper, immersing the paper encased steel in a celluloid solution, drying it by subjecting it to heat, cutting it into pieces of the desired length, and finishing the ends of the pieces thus formed by dipping them into a celluloid solution and then drying them.

55 8. The method of making corset boning which consists in encasing a ribbon-like piece of steel in a covering of paper, immersing the paper encased steel in a celluloid solution, drying it by subjecting it to heat, cutting it into pieces of the desired length, and finishing the ends of the pieces thus formed by covering them with metal tips and then dipping them into a celluloid solution, and then drying them.

60 9. Corset boning comprising a ribbon-like piece of steel encased in celluloid impregnated paper.

70 JOHN J. McCABE.